# EUROPEAN PATENT SPECIFICATION

(11) **EP 0 786 018 B1**
(45) Date of publication and mention of the grant of the patent: **09.01.2002**
(21) Application number: 95933529.0
(22) Date of filing: 11.10.1995
(51) Int. Cl.: C23F 11/10

(54) **CORROSION INHIBITING COMPOSITIONS**
KORROSIONSINHIBIERENDE ZUSAMMENSETZUNGEN
COMPOSITIONS INHIBANT LA CORROSION

(30) Priority: 11.10.1994 GB 9420478; 14.06.1995 GB 9512032
(43) Date of publication of application: 30.07.1997
(73) Proprietor: Great Lakes Chemical (Europe) GmbH, 8500 Frauenfeld (CH)
(72) Inventor: PATEL, Suresh, Manchester M27 5NJ (GB)
(74) Representative: McPherson, Alexander
(86) International application number: GB9502404
(87) International publication number: WO9611291

(56) References cited:
- EP-A- 0 009 080
- EP-A- 0 122 013
- EP-A- 0 360 746
- EP-A- 0 488 538
- EP-A- 0 516 346
- US-A- 4 717 542

## Description

This invention relates to compositions useful as additives for aqueous systems in order to inhibit the corrosion of metal surfaces which are in contact with these systems, to methods of inhibiting corrosion which comprise adding these novel compositions to aqueous systems and to aqueous systems which contain certain novel combinations of known corrosion inhibitors.

There have been a very large number of proposals to inhibit the corrosion of metal surfaces which are in contact with water which comprise adding various chemicals and formulated products to the aqueous system. A wide variety of products are used in this application. One class of compounds which are widely employed as corrosion inhibitor in aqueous systems are organic phosphonates and polyphosphonates. However, there remains a need for new products which are more effective or more cost effective in reducing corrosion.

USP 4689200 discloses the use of 2-hydroxy phosphono acetic acid or a water soluble salt thereof as an additive for aqueous systems in order to inhibit the corrosion of metal in contact with that aqueous system. This disclosure also suggests that the 2-hydroxy phosphono acetic acid may be used in conjunction with other known corrosion inhibitors. Among the many known corrosion inhibitors which are mentioned in this disclosure are phosphonic acids and their salts. USP 4689200 also proposes that the 2-hydroxy phosphono acetic acid may be used in conjunction with other additives and in particular scale inhibiting additives. Among many known scale inhibitors which are mentioned are the phosphino polycarboxylic acids which are described in British Patent 1458235. EPA 277412 describe a process for the reduction of corrosion of iron based metals in contact with aqueous systems which comprises adding combination of hydroxy phosphono acetic acid and water soluble 1-acrylamido-2-methyl propane sulphonic acid copolymer with acrylic or methacrylic acid to that aqueous system.

EPA 516346 discloses a process for the production of phosphono (co)telomers which are useful as scale inhibitors and corrosion inhibitors in aqueous systems. The telomeric portion of these compounds may be derived from a wide variety of olefinic compounds including 2-acrylamido-2-methyl propane sulphonic acid (AMPS) or from mixtures of such olefins including in particular mixtures of AMPS and acrylic acid. The use of these phosphonic (co)telomers in conjunction with other compounds known to be useful in the treatment of aqueous systems is also proposed. Amongst a very large number of such compounds which are mentioned as being known is 2-hydroxy phosphono acetic acid. EPA360746 discloses novel phosphono cotelomers which are useful inter alia as corrosion inhibitors. The use of these cotelomers in conjunction with other known corrosion inhibitors is also disclosed.

We have now discovered a particular phosphono cotelomer which interacts synergistically with known organophosphorus corrosion inhibitors which contain at least one phosphonic acid group as part of their molecular structure to provide improved corrosion inhibiting properties. Further since the phosphono cotelomer also exhibits scale inhibiting and dispersing activity the novel combination of these two materials is useful in the treatment of aqueous systems in order to inhibit scale formation and the deposition of particulate materials whilst at the same time inhibiting corrosion of metal surfaces.

The phosphono cotelomer which has been discovered to be useful in the compositions of this invention is that derived from a combination of acrylic acid and 2-acrylamido 2-methyl propane sulphonic acid (AMPS). The production of such a cotelomer is described in EPA 516346. However, there is no disclosure in the prior art of a composition comprising this cotelomer and an organophosphorus corrosion inhibitor.
Accordingly from one aspect this invention provides a composition useful as an additive to aqueous systems in order to inhibit the corrosion of metal surfaces in contact with that aqueous system which comprises:
(i) an organophosphorus corrosion inhibitor having the formula I or a water soluble salt thereof, in which R₃ may represent a group having the formula CO₂H, a group having the formula P(=O)(OH)₂, a group having the formula CH₂P(=O)(OH)₂, a group having the formula CH₂CH₂P(=O)(OH)₂ or a group having the formula NR₅R₆ in which R₅ and R₆ which may be the same or different represent a hydrogen atom; a methyl group; a group having the formula C[(R₇)₂]ₓP(=O)(OH)₂ or a group having the formula C[(R₇)₂]ₓCO₂H in which R₇ represents a hydrogen atom or a methyl group; and x is an integer having a value of 1 or 2;
   R₂ and R₄ which may be the same or different may represent a hydrogen atom, a hydroxyl group, an alkyl group comprising from 1 to 8 carbon atoms, a group having the formula -(CH₂)ₙCO₂H, where n is zero or an integer having a value of from 1 to 4, or an amine group having the formula -NH₂.

Preferably R₃ represents a group having the formula CO₂H or a group having the formula P(=O)(OH)₂; R₂ represents a hydrogen atom or a methyl group; and R₄ represents a hydroxyl group.
(ii) a phosphono cotelomer having the formula: and A represents a copolymeric residue containing at least one repeat unit having the formula III
wherein R₁ represents a hydrogen atom or a methyl group and at least one repeat unit having the formula IV or a water soluble salt thereof.

The phosphono telomer may be any compound of Formula II which is sufficiently water soluble to be effective. It may comprise repeat units of Formula III and repeat units of Formula IV in a wide range of proportions. The ratio of the number of units of formula III to the number of units of formula IV may vary from 99:1 to 1:99 but is more usually in the range 25:1 to 1:25. The most preferred polymers useful according to this invention are those wherein this ratio is in the range 20:1 to 2:1 ie, those which contain a greater proportion of the repeat unit having the formula III.

The cotelomers of formula II will typically have a molecular weight Mw of from 500 to 10,000 and more preferably of from 2,000 to 4,000. These cotelomers may be produced by a variety of processes which are known to the art. Generally these processes comprise the reaction of a monomer of formula III typically acrylic acid or methacrylic acid with the monomer of formula IV which is 2-acrylamido-2-methyl propane sulphonic acid (hereinafter for convenience AMPS) in the presence of a hypophosphite telogen. Such processes have been described in USP 4046707, EPA 150706, EPA 360746 and EPA 516346..The phosphonate telomers are preferably produced by the aqueous process which is described in EPA 516346. Such process typically comprise (a) the reaction of hypophosphorous acid or a hypophosphite with a carbonyl compound which is typically acetone, (b) reacting the product from (a) with the (meth)acrylic acid and the AMPS in the presence of a free radical initiator and converting the product of step (b) to the desired phosphonate (co)telomer by reaction eg, with hypochlorite. The process may vary according to the teachings of EPA 516346.

In particular a variety of carbonyl compounds may be employed in step (a) representative examples being formaldehyde, acetaldehyde, propionaldehyde, butyraldehyde, methylethyl ketone, diethyl ketone, dipropyl ketone, dibutyl ketone, cyclopentanone and cyclohexanone. The products obtained from these processes are aqueous solutions which may be used as such in the compositions or they may be purified prior to use. The phosphonate cotelomers are produced in their acid form and they may be wholly or partially neutralised prior to use.
Where the compositions of this inventions are added to alkaline media neutralisation may take place in situ and neutralisation at this production stage may thereby be irrelevant.

The second component of the compositions useful in this invention is an organophosphonate corrosion inhibitor having the general formula I. A number of such compounds are known and used in the art. A preferred group of phosphonates of formula I, which are useful according to this invention are those wherein at least one of the groups R₂ and R₄ represents a hydrogen atom. Particularly preferred phosphonates within this group include those wherein the other of the groups R₂ and R₄ also represents a hydrogen atom or a hydroxyl group -OH an amine group - NH₂ or a carboxylic acid group - CO₂H.

A second preferred group of compounds are those of the formula I wherein R₃ represents -CO₂H or PO(OH₂).

The most preferred phosphonates for use in the present invention are generally those which are in use or have been proposed to be useful as corrosion inhibitors in aqueous media.

Specific examples of these phosphonates include 2-hydroxyphosphono acetic acid, hydroxyethylidene diphosphonic acid (HEDP), hydroxy propylidene diphosphonic acid, hydroxy isobutylidene diphosphonic acid, 2-phosphono butane-1,2,4 tricarboxylic acid, amino tris(methylene phosphonic acid), diethylene triamino penta (methylene phosphonic acid), phosphonoacetic acid, 2-phosphonopropionic acid, 2-phosphonoheptanoic acid, 2-hydroxy-2-methyl phosphonoacetic acid, 2-hydroxy-2-butyl phosphonoacetic acid, 3-phosphono-3-hydroxy butyric acid, 2-phosphonoethane-1,2-dicarboxylic acid, methane diphosphonic acid, 1,2-ethanediphosphonic acid, 1,3-propane- diphosphonic acid, hydroxymethyl diphosphonic acid, 2-amino-phosphonoacetic acid, 2-amino-2-methyl phosphonoacetic acid, nitrilo-tris- methylene phosphonic acid, methylamino-bis-methylene phosphonic acid and phosphonomethyl glycine. Any of these phosphates may be useful according to this invention.

Preferred phosphonates are 2-hydroxyphosphono acetic acid, hydroxyethylidene diphosphonic acid and 2-phosphonobutane 1,2,4 tricarboxylic acid. 2-hydroxyphosphono acetic acid has been described in USP 3032500 and EPA 0050792. It can be prepared by known methods eg, by reacting orthophosphorous acid, a salt or a solution thereof, or phosphorus trichloride with glyoxylic acid or a salt or a solution thereof. Hydroxyethylidene disphosphonic acid and 2- phophono butane, 1, 2,4 tricarboxylic acid are also articles of commerce which are widely used as corrosion inhibitors in aqueous media.

The phosphonate corrosion inhibitors may be used as the free acid or as a wholly or partially neutralised salt thereof. Examples of suitable salts include the lithium, sodium, potassium, calcium, strontium, magnesium, ammonium, methylamine, ethylamine, n-propylamine, triethylamine, n-butylamine, n-hexylamine, octylamine, ethanolamine, diethanolamine, triethanolamine and morpholine salts.

The mixtures of phosphonate corrosion inhibitors and the phosphono cotelomers exhibit synergy over the entire range of proportions. Thus the ratio of the weight of one to the weight of the other may vary from 99:1 to 1:99. However, in general we prefer they are employed in proportions in which the weight ratio of phosphonate to phosphono cotelomer lies in the range 4:1 to 1:4. The proportions used in a particular application will be chosen so as to balance the benefits of performance against cost. When the phosphonate is 2-hydroxyphosphonoacetic acid the proportion of 2-hydroxyphosphonoacetic acid will generally be increased to provide a greater degree of corrosion inhibition. However, where a cost effective corrosion inhibitor is required it may be preferred to utilise a higher proportion of the phosphono cotelomer as this is the less costly component of the mixture.

The amount of the mixture which is added to an aqueous medium will generally be the same as is currently known in the art. Typically the mixture will be added so as to result in a concentration of from 0.1 to 50,000 ppm of the mixture of additives in the aqueous system. More usually this concentration will be in the range 0.5 to 100 ppm and most preferably will be in the range 1.0 to 50 ppm.

The phosphonate and the phosphono cotelomers are generally compatible and may be mixed together prior to their addition to an aqueous system. The addition of such mixtures to aqueous systems which are in contact with a metal surface in order to inhibit the corrosion of that surface constitutes a further aspect of the invention. The phosphonate and the phosphono cotelomer may be added separately to aqueous systems and processes involving this separate addition constitute a further aspect of the invention.

The phosphonate and phosphonate cotelomers may be used in combination to inhibit corrosion in soft waters (typically containing less than 30ppm calcium ions) and hard waters (typically containing say 100ppm, or more) of calcium ions.

The mixture of compounds of this invention may be used alone, or in conjunction with other compounds known to be useful in the treatment of aqueous systems.

In the treatment of systems which are completely aqueous, such as cooling water systems, air-conditioning systems, steam-generating systems, sea-water evaporator systems, hydrostatic cookers, and closed circuit heating or refrigerant systems, further corrosion inhibitors may be used such as, for example, water soluble zinc salts; phosphates; polyphosphates; nitrates, for example, sodium nitrate; nitrites, eg, sodium nitrite; molybdates, eg, sodium molybdate, tungstates eg, sodium tungstate; silicates, eg, sodium silicate; benzotriazole, bis-benzotriazole or copper deactivating benzotriazole or tolutriazole derivatives eg, their Mannich base derivatives; mercaptobenzotriazole; N-acyl sarcosines especially sodium N-lauryl sarcosinate; N-acylimino diacetic acids; alkanolamines especially the ethanolamines; fatty amines; and organic acids, for example, polymaleic acid and benzoic acid, p-tert-butyl benzoic acid, disodim sebacate, triethanolamine laurate, iso-nonanoic acid.
Moreover, in such completely aqueous systems, the inhibitor used according to the invention may be used in conjunction with further dispersing and/or threshold agents, eg,polymaleic acid polymerised acrylic acid (or its salts), eg, copolymers of acrylic acid and hydroxyalkylated acrylic acid, and substituted derivatives of polymaleic and polyacrylic acids and their copolymers, phosphino- polycarboxylic acids (as described in British Patent 1458235), the cotelomeric compounds described in European Patent Application 150706, hydrolysed polyacrylonitrile, polymerised methacrylic acid and its salts, polyacrylamide and copolymers thereof with acrylic and methacrylic acids, lignin sulphonic acid and its salts, tannin, napthalene sulphonic acid/formaldehyde condensation products, starch and its derivatives, cellulose, acrylic acid/lower alkyl hydroxyacrylate copolymers, eg, those described in US Patent Specification No: 4029577, styrene/maleic anhydride copolymers and sulphonated styrene homopolymers, eg, those described in US Patent Specification No: 4374733 and combinations thereof.

Other agents which may be incorporated into water treatment compositions or this convention include precipitating agents such as alkali metal orthophosphates, carbonates: oxygen scavengers such as alkali metal sulphites and hydrazines; sequestering agents such as nitrilotriacetic acid and its salts; antifoaming agents such as silicones, eg, polydimethylsiloxanes, distearylsebacamide, distearyl adipamide and related products derived from ethylene oxide and/or propylene oxide condensations, fatty alcohols such as capryl alcohols and their ethylene oxide condensates and biocides, eg, amines, quaternary ammonium compounds, chloro-phenols, sulphur-containing compounds such as sulphones, methylene bis thiocyanates and carbamates, isothiazolones, brominated propionamides, triazines, phosphonium compounds, chlorine and chlorine-releasing agents, bromine and bromine releasing agents and organometallic compounds such as tributyl tin oxide.

If the system to be treated by the method of the invention is not completely aqueous, eg, an aqueous machining fluid formulation, it may be eg, a water dilutable cutting or grinding fluid.

The aqueous machining fluid formulations of the invention may be eg, metal working formulations. By "metal working", we mean reaming, broaching, drawing, spinning, cutting, grinding, boring, milling, turning, sawing, non-cutting shaping or rolling. Examples of water-dilutable cutting or grinding fluids into which the corrosion inhibiting combinations of this invention may be incorporated include
a) aqueous concentrates of one or more corrosion inhibitors, and optionally one or more anti-wear additives, used at dilutions of 1:50 to 1:100, which are usually employed as grinding fluids;
b) polyglycols containing biocides, corrosion inhibitors and anti-wear additives which are used at dilutions of 1:20 to 1:40 for cutting operations and 1:60 to 1:80 for grinding;
c) semi-synthetic cutting fluids similar to (b) but containing in addition 10 to 25% oil with sufficient emulsifier to render the water diluted product translucent;
d) an emulsifiable mineral oil concentrate containing, for example, emulsifiers, corrosion inhibitors, extreme pressure/antiwear additives, biocides, anti-foaming agents, coupling agents etc; they are generally diluted from 1:10 to 1:50 with water to a white opaque emulsion;
e) a product similar to (d) containing less oil and more emulsifier which, on dilution to the range 1:50 to 1:100, gives a translucent emulsion for cutting or grinding operations.

For those partly-aqueous systems in which the aqueous system component is an aqueous machining fluid formulation, the synergistic mixtures according to the invention may be used as such, or in admixture with other additives, eg, known further corrosion inhibitors and/or extreme-pressure additives.

Examples of other corrosion inhibitors which may be used in these aqueous systems, in addition to the inhibitor composition used according to the invention, include the following groups:
a) Organic acids, their esters or ammonium, amine, alkanol-amine and metal salts, for example, benzoic acid, p-tert-butyl benzoic acid, disodium sebacate, triethanolamine laurate, iso-nonanoic acid, triethanolamine salt of (p-toluene sulphonamido caproic acid), triethanolamine salt of benzene sulphonamido caproic acid, triethanolamine salts of 5-ketocarboxylic acid derivatives as described in European Patent No: 41927, sodium N-lauroyl sarcosinate or nonyl phenoxy acetic acid;
b) Nitrogen containing materials such as the following types: fatty acid alkanolamides; imidazolines, for example, 1-hydroxy-ethyl-2-oleyl-imidazolines; oxazolines; triazoles for example, benzotriazoles, or their Mannich base derivatives; triethanolamines; fatty amines; inorganic salts, for example, sodium nitrate; and the carboxy-triazine compounds described in European Patent Applications No: 46139;
c) Sulphur containing compounds such as the following types: sodium, calcium or barium petroleum sulphonates, or heterocyclics, for example, sodium mercaptobenzothiazole. Nitrogen containing materials, particularly triethanolamine, are preferred.

Examples of extreme pressure additives which may be present in the systems treated according to the present invention include sulphur and/or phosphorus and/or halogen containing materials, for instance, sulphurised sperm oil, sulphurised fats, tritolyl phosphate, chlorinated paraffins or ethoxylated phosphate esters.

The partly-aqueous system treated by the method of the present invention may also be aqueous surface-coating compositions, eg emulsion paints and aqueous coatings for metallic substrates.

The aqueous surface-coating composition may be, eg, a paint such as styrene-acrylic copolymer emulsion paint, a resin, latex, or other aqueous based polymer surface-coating systems, to coat a metal substrate. The inhibitor composition used according to the invention may be employed to prevent flash rusting of the metal substrate during application of the surface coating and to prevent subsequent corrosion during use of the coated metal.

In aqueous surface-coating compositions treated by the method of the invention the inhibitor composition may be used singly, or in admixture with other additives, eg, known corrosion inhibitors, biocides, emulsifiers and/or pigments.

Examples of biocides which may be used in these aqueous systems include the following:

Phenols, and alkyl and halogenated phenols, for example, pentachlorophenol, o-phenylphenol, o-phenyoxyphenol and chlorinated o-phenoxyphenol, and salicylanilides, diamines, triazines and organometallic compounds such as organomercury compounds and organotin compounds.

Examples of pigments which may be used in these aqueous systems include titanium dioxide, zinc chromate, iron oxide and organic pigments such as the phthalocyanines.

### The invention is illustrated by the following example:

### Example One

A corrosion test was carried out assessing the ability of various blends of 2-hydroxyphosphonoacetic acid, hydroxyethylidene diphosphonic acid and 2-phosphonobutane 1,2,4-tricarboxylic acid (A) with a phosphonated (co)telomer having a molecular weight of 2000 to 3000 derived from acrylic acid and AMPS (B) in the following water:

| | |
|---|---|
| Calcium ions | 150 ppm as CaCO₃ |
| Magnesium ions | 75 ppm as CaCO₃ |
| Total Alkalinity | 350 ppm as CaCO₃ |
| Chloride ions | 200 ppm as Cl⁻ ion |
| Sulphate ions | 200 ppm as SO₄ ion |
| pH | 8 |

The test is carried out by using two cleaned and pre-weighed mild steel coupons which are secured to a stainless steel shaft by means of a threaded PTFE holder. The coupons are then rotated at 150 rpm for 42 hours at 40°C in the above aerated water with the additive present at a total concentration of 20 ppm (actives). The aeration rate used is 1 litre per minute per test.

After 42 hours the coupons are removed, cleaned and weighed and the corrosion rate was calculated using equation below.$\frac{\text{Weight loss of 2 coupons (mg)}}{{\text{Surface area of 2 coupons (dm}}^{\text{2}} \text{)x Time (days)}} \text{= Corrosion rate (mdd)}$
Corrosion rate (mdd)x 0.183 (factor for mild steel from the density of mild steel) = mpy
mdd = milligrams weight loss/dm²/day
mpy = Mls per year
Mls = 1/1000 th inch

The lower the corrosion rate (mdd) or mpy the better the protection to corrosion of mild steel by the additive.

The results are shown in figures 1, 2 and 3.

## Claims

1. A composition useful as an additive to aqueous systems in order to inhibit the corrosion of metal surfaces in contact with that aqueous system which comprises:
(i) an organophosphorus corrosion inhibitor having the formula I or a water soluble salt thereof, in which R₃ may represent a group having the formula CO₂H, a group having the formula P(=O) (OH)₂, a group having the formula CH₂P(=O)(OH)₂, a group having the formula CH₂CH₂P(=O)(OH)₂ or a group having the formula NR₅R₆ in which R₅ and R₆ may be the same or different represent a hydrogen atom; a methyl group; a group having the formula C[(R₇)₂]ₓP(=O)(OH)₂ or a group having the formula C[(R₇)₂]ₓCO₂H in which R₇ represents a hydrogen atom or methyl group; and x is an integer having a value of 1 or 2;
R₂ and R₄ which may be the same or different may represent a hydrogen atom, a hydroxyl group, an alkyl group comprising from 1 to 8 carbon atoms, a group having the formula -(CH₂)ₙCO₂H, where n is zero or an integer having a value of from 1 to 4. or an amine group having the formula NH₂
(ii) a phosphono cotelomer having the formula: and A represents a copolymeric residue containing at least one repeat unit having the formula III
wherein R₁ represents a hydrogen atom or a methyl group
and at least one repeat unit having the formula IV or a water soluble salt thereof.

2. A composition according to claim 1 **characterised in that** R₃ represents a group -CO₂H.

3. A composition according to either of claims 1 or 2 **characterised in that** R₃ represents a group P(=O)(OH)₂.

4. A composition according to any of the preceding claims **characterised in that** R₂ represents a hydrogen atom.

5. A composition according to any of the preceding claims **characterised in that** R₄ represents a hydroxyl group.

6. A composition according to claim 1 **characterised in that** the phosphono cotelomer has a molecular weight Mw of from 500 to 10,000.

7. A composition according to claim 6 **characterised in that** the phosphono cotelomer has a molecular weight of from 2,000 to 4,000.

8. A composition according to any of the preceding claims **characterised in that** R₁ represents a hydrogen atom.

9. A composition according to any of the preceding claims **characterised in that** the ratio of the number of repeat units of formula III to the number of repeat units of formula IV is from 25:1 to 1:25.

10. A composition according to claim 9 **characterised in that** the ratio of the number of repeat units of formula III to the number of repeat units of formula IV is in the range 20:1 to 2:1.

11. A composition according to any of the preceding claims **characterised in that** the organophosphorus corrosion inhibitor is selected from the group comprising 2-hydroxyphosphonoacetic acid, hydroxyethylidene diphosphonic acid, hydroxypropylidene diphosphonic acid, hydroxybutylidene diphosphonic acid, hydroxyisobutylidene diphosphonic acid, 2-phosphonobutane 1,2,4-tricarboxylic acid, amino tris(methylene phosphonic acid) and diethylene triamino penta (methylene phosphonic acid).

12. A composition according to claim 11 **characterised in that** the organophosphorus corrosion inhibitor is selected from the group comprising 2-hydroxyphosphonoacetic acid, hydroxy ethylidene diphosphonic acid and 2-phosphonobutane 1,2,4-tricarboxylic acid.

13. A composition according to either of claims 11 or 12 **characterised in that** the organophosphorus corrosion inhibitor is 2-hydroxyphosphonoacetic acid.

14. A composition according to any of the preceding claims **characterised in that** the ratio of the weight of the organophosphorus corrosion inhibitor to the weight of the phosphono cotelomer is in the range 99:1 to 1:99.

15. A composition according to claim 14 **characterised in that** the ratio of the weight of the organophosphorus corrosion inhibitor to the weight of phosphono cotelomer is in the range 4:1 to 1:4.

16. A method for inhibiting the corrosion of a metal surface which is in contact with an aqueous system **characterised in that** an effective quantity of a mixture according to any of claims 1 to 15 is added to the aqueous system.

17. A method according to claim 16 **characterised in that** the mixture of the organophosphorus corrosion inhibitor and the phosphono cotelomer is produced by their separate addition to the aqueous system.

18. A method according to claim 16 **characterised in that** the aqueous system contains from 0.1 to 50,000 ppm of a mixture according to any of claims 1 to 15.

19. A method according to any of the preceeding claims **characterised in that** the aqueous system comprises at least 100ppm of calcium ions.

20. A method according to any of claims 16 to 19 **characterised in that** the aqueous system comprises less than 300 ppm of calcium ions.

21. An aqueous system which comprises a mixture according to any of claims 1 to 15.

22. A system according to claim 21 which comprises from 0.1 to 50,000 ppm of the mixture.

## Patentansprüche

1. Zusammensetzung, nützlich zur Verwendung als Additiv zu wässrigen Systemen zur Unterdrückung der Korrosion von Metalloberflächen, die mit diesem wässrigen System in Kontakt stehen, welche umfasst:
(i) einen phosphororganischen Korrosionsinhibitor mit der Formel I: oder ein wasserlösliches Salz davon, in der R₃ eine Gruppe darstellen kann mit,der Formel CO₂H, eine Gruppe mit der Formel P(=O)(OH)₂, eine Gruppe mit der Formel CH₂P(=O)(OH)₂, eine Gruppe mit der Formel CH₂CH₂P(=O)(OH)₂ oder eine Gruppe mit der Formel NR₅R₆, in der R₅ und R₆ gleich oder unterschiedlich sein können und ein. Wasserstoffatom, eine Methylgruppe, eine Gruppe mit der Formel C[(R₇)₂]ₓP(=O)(OH)₂ oder eine Gruppe mit der Formel C[(R₇)₂]ₓCO₂H darstellen, in der R₇ ein Wasserstoffatom oder eine Methylgruppe darstellt; und x eine ganze Zahl mit einem Wert von 1 oder 2 ist.
R₂ und R₄, die gleich oder verschieden sein können, können ein Wasserstoffatom, eine Hydroxylgruppe, einen Alkylrest, umfassend 1 bis 8 Kohlenstoffatome, eine Gruppe der Formel -(CH₂)ₙCO₂H, wobei n 0 oder eine ganze Zahl mit einem Wert von 1 bis 4 ist, oder eine Amingruppe mit der Formel NH₂ darstellen können,
(ii) ein Phosphon-Cotelomer mit der Formel: und A einen Copolymerrest darstellt, der mindestens eine Wiederholungseinheit mit der Formel III enthält
worin R₁ ein Wasserstoffatom oder eine Methylgruppe darstellt und mindestens eine Wiederholungseinheit mit der Formel IV oder ein wasserlösliches Salz davon.

2. Zusammensetzung gemäß Anspruch 1, **dadurch gekennzeichnet, dass** R₃ eine -CO₂H-Gruppe darstellt.

3. Zusammensetzung gemäß einem der Ansprüche 1 oder 2, **dadurch gekennzeichnet, dass** R₃ eine P(=O)(OH)₂-Gruppe darstellt.

4. Zusammensetzung gemäß einem der vorstehenden Ansprüche, **dadurch gekennzeichnet, dass** R₂ ein Wasserstoffatom darstellt.

5. Zusammensetzung gemäß einem der vorstehenden Ansprüche, **dadurch gekennzeichnet, dass** R₄ eine Hydroxylgruppe darstellt.

6. Zusammensetzung gemäß Anspruch 1, **dadurch gekennzeichnet, dass** das Phosphon-Cotelomer ein Molekulargewicht Mw von 500 bis 10000 hat.

7. Zusammensetzung gemäß Anspruch 6, **dadurch gekennzeichnet, dass** das Phosphon-Cotelomer ein Molekulargewicht von 2000 bis 4000 hat.

8. Zusammensetzung gemäß einem der vorstehenden Ansprüche, **dadurch gekennzeichnet, dass** R₁ ein Wasserstoffatom darstellt.

9. Zusammensetzung gemäß einem der vorstehenden Ansprüche, **dadurch gekennzeichnet, dass** das Verhältnis der Zahl der Wiederholungseinheiten der Formel III zu der Zahl der Wiederholungseinheiten der Formel IV von 25:1 bis 1:25 liegt.

10. Zusammensetzung gemäß Anspruch 9, **dadurch gekennzeichnet, dass** das Verhältnis der Zahl der Wiederholungseinheiten der Formel III zu der Zahl der Wiederholungseinheiten der Formel IV im Bereich 20:1 bis 2:1 liegt.

11. Zusammensetzung gemäß einem der vorstehenden Ansprüche, **dadurch gekennzeichnet, dass** der phosphororganische Korrosionsinhibitor ausgewählt wird aus 2-Hydroxyphosphonessigsäure, Hydroxyethylidendiphosphonsäure, Hydroxypropylidendiphosphonsäure, Hydroxybutylidendiphosphonsäure, Hydroxy:isobutylidendiphosphonsäure, 2-Phosphonbutan-1,2,4-tricarbonsäure, Aminotris(methylenphosphonsäure) und Diethylentriaminopenta(methylenphosphonsäure).

12. Zusammensetzung gemäß Anspruch 11, **dadurch gekennzeichnet, dass** der phosphororganische Korrosionsinhibitor ausgewählt wird aus 2-Hydroxyphosphonessigsäure, Hydroxyethylidendiphosphonsäure und 2-Phosphonbutan-1,2,4-tricarbonsäure.

13. Zusammensetzung gemäß einem der Ansprüche 11 oder 12, **dadurch gekennzeichnet, dass** der phosphororganische Korrosionsinhibitor 2-Hydroxyphosphonessigsäure ist.

14. Zusammensetzung gemäß einem der vorstehenden Ansprüche, **dadurch gekennzeichnet, dass** das Verhältnis des Gewichts des phosphororganischen Korrosionsinhibitors zu dem Gewicht des Phosphon-Cotelomers im Bereich von 99:1 bis 1:99 liegt.

15. Zusammensetzung gemäß Anspruch 14, **dadurch gekennzeichnet, dass** das Verhältnis des Gewichts des phosphororganischen Korrosionsinhibitors zu dem Gewicht des Phosphon-Cotelomers im Bereich von 4:1 bis 1:4 liegt.

16. Verfahren zur Hemmung der Korrosion einer Metalloberfläche, die mit einem wässrigen System in Kontakt steht, **dadurch gekennzeichnet, dass** dem wässrigen System eine wirksame Menge eines Gemisches gemäß einem der Ansprüche 1 bis 15 zugegeben wird.

17. Verfahren gemäß Anspruch 16, **dadurch gekennzeichnet, dass** das Gemisch aus dem phosphororganischen Korrosionsinhibitor und dem Phosphon-Cotelomer durch ihre getrennte Zugabe zu dem wässrigen System hergestellt wird.

18. Verfahren gemäß Anspruch 16, **dadurch gekennzeichnet, dass** das wässrige System 0,1 bis 50000 ppm eines Gemisches gemäß einem der Ansprüche 1 bis 15 enthält.

19. Verfahren gemäß einem der vorstehenden Ansprüche, **dadurch gekennzeichnet, dass** das wässrige System mindestens 100 ppm Kalzium-Ionen umfasst.

20. Verfahren gemäß einem der Ansprüche 16 bis 19, **dadurch gekennzeichnet, dass** das wässrige System weniger als 300 ppm Kalzium-Ionen umfasst.

21. Wässriges System, das ein Gemisch gemäß einem der Ansprüche 1 bis 15 umfasst.

22. System gemäß Anspruch 21, das 0,1 bis 50000 ppm des Gemisches umfasst.

## Revendications

1. Composition utile comme additif à des systèmes aqueux afin d'inhiber la corrosion de surfaces métalliques en contact avec ledit système aqueux qui comprend :
(i) un inhibiteur de corrosion organophosphoré de formule I ou un sel soluble dans l'eau de celui-ci, dans laquelle R₃ peut représenter un groupe de formule CO₂H, un groupe de formule P(=O)(OH)₂, un groupe de formule CH₂P(=0) (OH)₂, un groupe de formule CH₂CH₂P(=0) (OH)₂ ou un groupe de formule NR₅R₆ dans lequel R₅ et R₆ peuvent être identiques ou différents et représentent un atome d'hydrogène, un groupe méthyle, un groupe de formule C[(R₇)₂]ₓP(=O)(OH)₂ ou un groupe de formule C[(R₇)₂]ₓCO₂H dans lequel R₇ représente un atome d'hydrogène ou un groupe méthyle, et x est un entier ayant une valeur de 1 ou 2 ;
R₂ et R₄ qui peuvent être identiques ou différents peuvent représenter un atome d'hydrogène, un groupe hydroxyle, un groupe alkyle comprenant de 1 à 8 atomes de carbone, un groupe de formule -(CH₂)ₙCO₂H, où n est égal à zéro ou est un entier ayant une valeur de 1 à 4, ou un groupe amine de formule NH₂
(ii) un cotélomère phosphonique de formule : et A représente un résidu copolymérique contenant au moins une unité répétée de formule III
dans laquelle R1 représente un atome d'hydrogène ou un groupe méthyle
et au moins une unité répétée de formule IV ou un sel soluble dans l'eau de celle-ci.

2. Composition selon la revendication 1 **caractérisée en ce que** R₃ représente un groupe -CO₂H.

3. Composition selon la revendication 1 ou 2 **caractérisée en ce que** R₃ représente un groupe P(=O)(OH)₂.

4. Composition selon l'une quelconque des revendications précédentes **caractérisée en ce que** R₂ représente un atome d'hydrogène.

5. Composition selon l'une quelconque des revendications précédentes **caractérisée en ce que** R₄ représente un groupe hydroxyle.

6. Composition selon la revendication 1 **caractérisée en ce que** le cotélomère phosphonique a une masse moléculaire Mw située entre 500 et 10.000.

7. Composition selon la revendication 6 **caractérisée en ce que** le cotélomère phosphonique a une masse moléculaire située entre 2.000 et 4.000.

8. Composition selon l'une quelconque des revendications précédentes **caractérisée en ce que** R₁ représente un atome d'hydrogène.

9. Composition selon l'une quelconque des revendications précédentes **caractérisée en ce que** le ratio du nombre d'unités répétées de formule III par rapport au nombre d'unités répétées de formule IV est de 25 : 1 à 1 : 25.

10. Composition selon la revendication 9 **caractérisée en ce que** le ratio du nombre d'unités répétées de formule III par rapport au nombre d'unités répétées de formule IV est situé dans une fourchette de 20 :1 à 2 :1.

11. Composition selon l'une quelconque des revendications précédentes **caractérisée en ce que** l'inhibiteur de corrosion organophosphoré est choisi parmi le groupe constitué de l'acide 2-hydroxyphosphonoacétique, de l'acide hydroxyéthylidène diphosphonique, de l'acide hydroxypropylidène diphosphonique, de l'acide hydroxybutylidène diphosphonique, de l'acide hydroxyisobutylidène diphosphonique, de l'acide 2-phosphonobutane 1,2,4-tricarboxylique, de l'acide amino tris (méthylène phosphonique) et de l'acide diéthylène triamino penta (méthylène phosphonique).

12. Composition selon la revendication 11 **caractérisée en ce que** l'inhibiteur de corrosion organophosphoré est choisi parmi le groupe constitué de l'acide 2-hydroxyphosphonoacétique, de l'acide hydroxyéthylidène diphosphonique et de l'acide 2-phosphonobutane 1,2,4-tricarboxylique.

13. Composition selon l'une quelconque des revendications 11 ou 12 **caractérisée en ce que** l'inhibiteur de corrosion organophosphoré est l'acide 2-hydroxyphosphonoacétique.

14. Composition selon l'une quelconque des revendications précédentes **caractérisée en ce que** le rapport de la masse de l'inhibiteur de corrosion organophosphoré par rapport à la masse du cotélomère phosphonique se situe entre 99:1 et 1:99.

15. Composition selon la revendication 14 **caractérisée en ce que** le rapport de la masse de l'inhibiteur de corrosion organophosphoré par rapport à la masse du cotélomère phosphonique se situe entre 4:1 et 1:4.

16. Procédé pour inhiber la corrosion d'une surface métallique qui est en contact avec un système aqueux **caractérisé en ce que** une quantité efficace d'un mélange selon l'une quelconque des revendications 1 à 15 est ajoutée au système aqueux.

17. Procédé selon la revendication 16 **caractérisé en ce que** le mélange de l'inhibiteur de corrosion organophosphoré et du cotélomère phosphonique est produit par leur addition séparée au système aqueux.

18. Procédé selon la revendication 16 **caractérisé en ce que** le système aqueux contient de 0,1 à 50.000 ppm d'un mélange selon l'une quelconque des revendications 1 à 15.

19. Procédé selon l'une quelconque des revendications précédentes **caractérisé en ce que** le système aqueux comprend au moins 100 ppm d'ions calcium.

20. Procédé selon l'une quelconque des revendications 16 à 19 **caractérisé en ce que** le système aqueux comprend moins de 300 ppm d'ions calcium.

21. Système aqueux qui comprend un mélange selon l'une quelconque des revendications 1 à 15.

22. Système selon la revendication 21 qui comprend entre 0,1 et 50.000 ppm du mélange.
